

## UNITED STATES PATENT OFFICE.

WILLIAM WARWICK STENNING, PERCY THOMAS WILLIAMS, WALTER HENRY BEASLEY, AND ARTHUR BERESFORD MIDDLETON, OF LONDON, ENGLAND, ASSIGNEES TO MINERALS SEPARATION NORTH AMERICAN CORPORATION, OF NEW YORK, N. Y., A CORPORATION.

## TREATMENT OF SMALL OR FINELY-DIVIDED COAL.

No Drawing.

Application filed November 11, 1922. Serial No. 600,407.

*To all whom it may concern:*

Be it known that we, WILLIAM WARWICK STENNING, PERCY THOMAS WILLIAMS, WALTER HENRY BEASLEY, and ARTHUR BERESFORD MIDDLETON, all British subjects, residing in London, in England, have invented certain new and useful Improvements in the Treatment of Small or Finely-Divided Coal, of which the following is a specification.

10 This invention consists in improvements in or relating to the treatment of small or finely divided coal to render it commercially utilizable, as in briquetting, and particularly to a process of treatment of coal by 15 coating with a flocculating medium the particles of coal suspended in a circuit liquor, whereupon the circuit liquor can readily be removed by the application of pressure. Such a process is described in United States 20 patent application Serial No. 404,106 filed 17th August 1920.

In such a process, when using a flocculating medium such as molten pitch, which is an effective binding agent, the coated coal 25 particles can eventually be pressed into strong briquettes, but when briquettes of this character are not required, other flocculating agents may be employed. In this case also, to facilitate handling, the treated 30 coal may be pressed into blocks which, although relatively soft, are sufficiently coherent and are herein referred to as briquettes.

The objects of the present invention are 35 to reduce the quantity of flocculating agent required, and to economize the amount of heat which may be needed in the preparation for briquetting. The term "circuit liquor" is employed herein to include water 40 or any other aqueous liquor in which the coal particles may be suspended during the treatment.

According to the present invention the coal particles are treated by agitation in a 45 circuit liquor together with finer coal particles which have been previously coated with a flocculating medium.

We have found that the fine coal particles, after being coated with a suitable medium

and flocculated, can be made to play the 50 part of a binding medium for coarser particles. The fine particles become attached to the coarse particles, the binding medium on the surface of the fine particles serving effectively to unite the whole together in 55 the subsequent operation of briquetting. We have found by experiment that the amount of binding medium required in such a treatment is considerably less than the amount required when the binding medium 60 is added to the aggregate of fine and coarse coal.

The invention includes a process for the treatment of finely-divided coal wherein fine coal particles are flocculated by agitation in 65 aqueous suspension with a flocculating medium and are subsequently mixed with coarser coal particles so as to flocculate the mixture and render the coal readily separable from associated water.

The invention further includes a process for the treatment of finely-divided coal wherein the coal is separated into fractions containing respectively coarser and finer particles, the finer particles are treated with 75 a flocculating medium and the coarser particles are thereupon suspended in circuit liquor and treated by agitation with the flocculated finer particles, with or without the further addition of a binding medium. 80 Preferably the finer particles are coated with the flocculating medium by agitating them, while in aqueous suspension, with the addition of the flocculating medium.

We have found that the heat consumed 85 during the briquetting process can be economized, because the coal originally suspended in cold circuit liquor, can be flocculated by treatment in the cold so as to be separated from that liquor or at least from 90 a substantial part thereof, and if heat is necessary for the subsequent operations the introduction of cold circuit liquor along with the fine coal can be obviated or minimized.

The invention therefore includes a process for the treatment of finely-divided coal as set forth above, wherein the initial treat-

ment of the finer coal particles with the floculating medium is carried out in a cold circuit liquor by the use of an agent capable of producing flocculation in the cold, such as anthracene oil, tar or the like. Preferably, the fine coal after flocculation is separated from cold circuit liquor by mechanical means (for example filtration) and is thereafter treated with coarser coal in hot circuit liquor, flocculated and separated from the liquor which is reused for the treatment of further quantities of mixed fine and coarse particles.

Thus, according to one form of the present invention, the coal suspended in water or aqueous circuit liquor is treated by screening, classification, or the like known method to separate the fine coal suspended in the water or circuit liquor from the coarse coal, the fine coal is flocculated in the cold circuit liquor by the addition of a suitable oil, tar or mixture of tar and pitch or the like while the pulp is being subjected to agitation and/or aeration, the said fine coal is separated from cold circuit liquor by filtration or the like mechanical method, and the fine coal together with the coarse coal with or without a binder such as molten pitch or finely ground solid pitch are added to and mixed by agitation with a hot circuit liquor, and finally the hot circuit liquor is moved from the coal by filtration or pressure and again used, while the hot coal is converted into briquettes substantially free from water by pressure in a mould of suitable design.

The size of the coal particles and the selection of the proper ratio of fine and coarse particles will vary according to circumstances and in carrying out the present invention, the extent to which classification is carried may be varied so as to obtain the best economical results. We have found with the coals we have tried that when the coal to be treated will pass a screen of 10 meshes to the linear inch, the fines that will pass through a screen of 60-80 meshes to the linear inch should be separated; in such cases the fines removed usually amount to about 25% by weight of the total coal.

Apparently the fine particles should be present in sufficient quantity to cover or coat the surfaces of the coarser particles more or less closely, and the quantity of binder or flocculating agent required seems to be a function of the total surface of the finer particles which are to be coated with it. The total collective surface of the particles in a sample of finely divided coal can be estimated by sifting it into various grades and estimating the surface of each grade separately on the assumption that all the particles in a grade are of an average size and have a simple cubical or other probable shape.

Taking for example duff coal from Powell Duffryn Colliery in South Wales, crushed to

pass a 10 mesh screen, the following grading analysis has been found of a sample of 100 grammes of the concentrates obtained by subjecting the coal to froth-flotation:

70

| Screen.   | Weight.  | Surface exposed. |    |
|-----------|----------|------------------|----|
|           | Grammes. | Square inches.   |    |
| +20.....  | 39.6     | 277              | 75 |
| +60.....  | 36.3     | 552              |    |
| +100..... | 4.2      | 165              |    |
| +200..... | 9.1      | 632              |    |
| -200..... | 10.8     | 2,225            |    |

The weight of this coal of a larger size 80 than 60 mesh is 75.9 grammes with an estimated surface of 829 square inches, and the weight of the coal smaller than 60 mesh is 24.1 grammes with an estimated surface of 3022 square inches.

By using a binder consisting of three parts of hard coal-tar pitch and two parts of by-product coke-oven tar obtained from the Bargoed Coke Ovens, South Wales, it is found that the whole of this coal mixed together and treated in an aqueous pulp by agitation with aeration, the binder being added in liquefied form, requires 7% of binder to produce effective flocculation of the particles which will lead to the production 95 of a first class briquette when subjected to proper pressure in a suitable mould.

Treating the coal, however, according to the present invention, the fines of a size smaller than 60 mesh are separated by treating the 100 concentrates in the form of a mobile pulp on a screen or sieve of 60 meshes to the linear inch. The finer particles which pass through the screen with the water amount by weight to about one-quarter of the coal concentrates. 105 The coarser particles are by this step separated from the bulk of the water. The separated fines, suspended in water, are agitated with an amount of binder equal to 5% on the total weight of the coal. Treatment is 110 carried out in a heated circuit liquor and the binder is added in a liquefied condition. After flocculation of the fines in this way the coarser particles, larger than 60 mesh and comprising 75.9% by weight of the coal are 115 admixed with the coated and flocculated finer particles. Flocculation results of the whole mass, and on subjecting this to pressure in a briquetting press a briquette results of equal quality with that which required 120 7% of binder when the whole of the coal was treated together in one step.

It seems evident that in this particular case 5% of binder is sufficient to cover effectively 3022 square inches of surface exposed on the portion of the coal smaller than 60 mesh, but is insufficient to cover effectively 3851 square inches exposed on the total product. Furthermore, apparently the quantity of binder required is approxi- 130

mately proportional to the exposed surface which it is required to coat directly. At the same time the amount of fines initially treated cannot be indefinitely reduced, as a sufficient quantity must be used to coat the coarser particles and act as an efficient binder or matrix therefor. The surface of the fines should in practice apparently be at least three times greater than the surface of the coarser particles for the best results.

Many reagents, other than the mixture of pitch and tar referred to above, may be used to flocculate the fine coal, and in some cases after flocculation of the fines an additional agent may be added when treating fines and coarse together. This is particularly the case where the agent used for the fines is one which will not lead to the production of briquettes of the desired strength. In practice, for briquetting purposes, it is always necessary to select an agent which helps, or at least does not hinder the final briquetting operation. Such agents are the coal-tar product known as anthracene oil, or an oil containing a substantial proportion of naphthalene or phenanthrene; the amount of such oil that it is permissible to use is limited by the condition that the use of too much oil produces weak briquettes; we have found that a quantity of anthracene oil amounting to 1% of the total weight of coal will serve to flocculate the fines, and an excellent briquette can be formed by adding the separated fine and coarse coal together with molten pitch, finely divided hard pitch or similar binder amounting to 4% of the total weight of coal, and mixing the whole in a circuit liquor at 80° to 100° C.

The following alternative procedure, using the same coals above described, illustrates the use of anthracene oil. As before, the coal is ground to pass a 10 mesh screen and subjected to concentration by the froth-flotation process for the removal of ash. The concentrate is still mixed with water, and in the form of a mobile pulp it is treated on a screen or sieve of 60 or 80 meshes to the linear inch. The fines are thereby separated, with the bulk of the water, in amount as before of about one-quarter by weight of the coal concentrates.

The aqueous suspension of finer particles (which is not heated) is introduced into an agitation apparatus, preferably an apparatus of the general type employed for agitating the pulp in the froth-flotation process, i. e., an apparatus which affords both agitation and aeration. During the agitation there is added to the pulp a small proportion, say 1%, of anthracene oil, this percentage being measured on the total weight of coal. By this process the finer particles become coated with the oil and flocculated, and can therefore be re-

moved from the cold liquor by settlement 65 and decantation, or by screening, or by filtration.

The final preparation of all the coal is effected in a hot circuit liquor which is used repeatedly. The coarser particles, substantially free from water, are added to the hot circuit liquor at 80° C. and the flocculated finer particles are also added, together with 70 4% of molten pitch or finely divided solid pitch measured on the total weight of coal. 75 The mixture is effected during agitation, preferably with aeration.

When the coated finer particles have had adequate opportunity of becoming attached to the coarse particles, the solid matter as a 80 whole is separated from the hot circuit liquor, again by settlement and decantation, or screening, or filtration, and the solid matter is directly subjected to briquetting, say in a 85 briquetting press.

The following example gives the results in detail obtained upon coal from the Saar Valley in France. The coal consisted of a mixture of bright and dull coal together with carbonaceous shale. The ash content 90 was 24.97% but this was reduced by flotation concentration to 9.12%.

This concentrate was screened to separate fines of a size such as to pass an aperture of 0.008 inch in linear dimensions and the finer 95 portion was treated in an acid circuit liquor containing 1 lb. sulphuric acid per ton of coal. The treatment was carried out in a cell provided with an agitator of the type used in the froth-flotation process, i. e., a cell provided with an agitator which gives vigorous agitation and aeration. A binding medium was added containing three parts of pitch and two parts of tar in the proportion of 5% of binding medium on the total weight 100 of the coal (fine and coarse). Steam was then admitted and the temperature of the pulp was raised to 90° C. After the flocculation of the finer portion of the coal in this way, the coarse particles were added 105 during agitation, and the whole material was thus flocculated. Thereafter it was drained and briquetted under pressure of 2 tons per square inch. The briquettes were eventually coked for two hours at a temperature 110 gradually rising to 1040° C. and yielded a coke having a crushing strength 115 of 2430 lbs. per square inch.

It will be noted that in this test the whole of the binding medium was employed in the 120 initial operation on the fines, and the treatment of the fines was therefore concluded in a hot circuit, owing to the large proportion of pitch in the binder. It has, however, already been pointed out that the use of a hot 125 circuit for the fines is not essential.

In place of the mixture of tar and pitch a mixture of 1½ parts of naphthalene to

3½ parts of pitch can be employed, the quantity amounting as before, to 5% of the total weight of the coal.

What we claim as our invention, and desire to secure by Letters Patent is:

1. A process for the treatment of finely-divided coal wherein the coal particles are treated by agitation in a circuit liquor together with finer coal particles which have previously been coated with a flocculating medium.
2. A process for the treatment of finely-divided coal wherein the coal particles are treated by agitation with aeration in a circuit liquor together with finer coal particles which have previously been coated with a flocculating medium.
3. A process for the treatment of finely-divided coal wherein fine coal particles are flocculated by agitation in aqueous suspension with a flocculating medium and are subsequently agitated in aqueous suspension with coarser coal particles so as to flocculate the mixture and render the coal readily separable from associated water.
4. A process for the treatment of finely-divided coal wherein the coal is separated into fractions containing respectively coarser and finer particles, the finer particles are treated with a flocculating medium and the coarser particles are thereupon suspended in circuit liquor and agitated so as to be flocculated with the treated finer particles.
5. A process for the treatment of finely-divided coal wherein fine coal particles are flocculated by agitation in aqueous suspension with a flocculating medium and are subsequently agitated in aqueous suspension with coarser coal particles so as to flocculate the mixture and render the coal readily separable from associated water with the further addition of a liquefied binding medium.
6. A process for the treatment of finely-divided coal wherein the coal is separated into fractions containing respectively coarser and finer particles, the finer particles are coated with a flocculating medium by agitating them, while in aqueous suspension, with the addition of the flocculating medium, and the coarser particles are thereupon suspended in circuit liquor and agitated so as to be flocculated with the coated finer particles.
7. A process for the treatment of finely-divided coal wherein fine coal particles are flocculated by agitation in aqueous suspension at normal atmospheric temperature with an agent capable of producing flocculation at that temperature and are subsequently agitated in aqueous suspension with coarser coal particles so as to flocculate the mixture and render the coal readily separable from associated water.
8. A process for the treatment of finely-divided coal wherein fine coal particles are flocculated by agitation in aqueous suspension at normal atmospheric temperature with an oily coal tar product and are subsequently agitated in aqueous suspension with coarser coal particles so as to flocculate the mixture and render the coal readily separable from associated water.
9. A process for the treatment of finely-divided coal wherein fine coal particles are flocculated by agitation in aqueous suspension at normal atmospheric temperature with anthracene oil and are subsequently agitated in aqueous suspension with coarser coal particles so as to flocculate the mixture and render the coal readily separable from associated water.
10. A process for the treatment of finely-divided coal wherein fine coal particles are flocculated by agitation in aqueous suspension at normal atmospheric temperature with an agent capable of producing flocculation at that temperature, are separated from cold circuit liquor, and are thereupon agitated with coarser coal particles in a heated circuit liquor with the addition of a liquefied binding medium so as to flocculate the mixture and render it readily separable from associated water.
11. A process for the treatment of finely-divided coal wherein fine coal particles are flocculated by agitation in aqueous suspension at normal atmospheric temperature with an agent capable of producing flocculation at that temperature, are separated from cold circuit liquor, are thereupon agitated with coarser coal particles in a heated circuit liquor with the addition of a liquefied binding medium so as to flocculate the mixture and render it readily separable from associated water, and are subjected to pressure to expel water and produce briquettes.
12. A process for the treatment of finely-divided coal wherein fine coal particles are flocculated by agitation in aqueous suspension by the addition of a suitable reagent, are thereupon agitated with coarser coal particles in aqueous suspension so as to flocculate the mixture and render it readily separable from water and are subjected to pressure to expel water and produce briquettes.
13. A process for the treatment of finely-divided coal wherein coal particles are treated by agitation in a circuit liquor together with finer coal particles which have previously been coated with a flocculating medium and are subjected to pressure to expel water and produce briquettes.
14. A process for the treatment of finely-divided coal wherein fine coal particles are flocculated by agitation in aqueous suspension at normal atmospheric temperature with anthracene oil, are separated from cold

circuit liquor, are thereupon agitated with coarser coal particles in a heated circuit liquor with the addition of a liquefied binding medium so as to flocculate the mixture and 5 render it readily separable from associated water, and are subjected to pressure so as to expel water and produce briquettes.

15. A process for the treatment of finely divided coal wherein coal particles are treated 10 by agitation in a circuit liquor together with a sufficient quantity of finer coal particles which have previously been coated with a flocculating medium to substantially coat the coarser particles with finer ones 15 distributed over their surface, and to render the whole of the coal readily separable from water.

16. A process for the treatment of finely divided coal wherein relatively coarse coal 20 particles are treated by agitation in a circuit liquor together with finer coal particles in sufficient quantity to have a total surface at least three times greater than that of the coarse particles, the finer particles having 25 previously been coated on their surfaces with a flocculating medium, so as to render the whole of the coal readily separable from water.

17. A briquette consisting of coarser and 30 finer grades of coal particles, the finer particles being coated on their surfaces with a flocculating and binding medium and being distributed over the surfaces of the coarser particles in sufficient quantity to act as a 35 binder in uniting them together.

18. A fuel product consisting of coarser and finer grades of coal particles, the finer particles being coated on their surfaces with a flocculating and binding medium and being 40 distributed over the surfaces of the the

coarser particles in sufficient quantity to render the whole mass readily separable from water.

19. A fuel product consisting of coarser and finer coal particles in such ratio that the 45 total surface of the finer coal particles is more than three times the total surface of the coarser particles, the finer particles being coated on their surfaces with a flocculating and binding medium and distributed 50 over the surfaces of the coarser particles so as to render the whole mass readily separable from water.

20. A briquette consisting of coarser and finer coal particles in such ratio that the 55 total surface of the finer coal particles is more than three times the total surface of the coarser particles, the finer particles being coated on their surfaces with a flocculating 60 and binding medium and distributed over the surfaces of the coarser particles so as to act as a binder in uniting them together.

In testimony whereof we have signed our names to this specification in the presence of 65 two subscribing witnesses.

WILLIAM WARWICK STENNING.

PERCY THOMAS WILLIAMS.

WALTER HENRY BEASLEY.

ARTHUR BERESFORD MIDDLETON.

Witnesses to the signatures of William Warwick Stenning, Walter Henry Beasley, and Arthur Beresford Middleton:

RICHARD THOMAS M. LYNNE,

PHILIP JOHN BERESFORD.

Witnesses to the signature of Percy Thomas Williams:

GEO. C. BOLTON,

JOHN IVOR HARRIS.